

# United States Patent Office

3,314,785

Patented Apr. 18, 1967

1

3,314,785  
ALLOY

Leonard F. Yntema, Wadsworth, and Arthur B. Michael,  
Lake Forest, Ill., assignors to Fansteel Metallurgical  
Corporation  
No Drawing. Filed Feb. 5, 1957, Ser. No. 638,210  
7 Claims. (Cl. 75—174)

The present invention relates to alloys of columbium and more particularly to columbium alloys which, compared to substantially pure columbium metal, have greatly improved strength characteristics and resistance to oxidation at elevated temperatures of the order of 1300° C. and higher.

Substantially pure columbium metal has many desirable properties which make it potentially useful as a structural metal at high temperatures. Thus, for example, it has a melting point of about 2450° C. and it possesses the same strength properties at elevated temperatures (of the order of 1300° C. and higher) as pure molybdenum, the refractory metal generally used heretofore for high temperature applications. In contrast to molybdenum, which cannot be worked at room temperature, but must be hot-worked, the refractory metal columbium can be cold worked. Columbium is thus easier to fabricate and can be formed into more complicated shapes than molybdenum. In addition, the extreme embrittling characteristics of molybdenum in use is not a characteristic of columbium. Unlike molybdenum welds, columbium welds are ductile and are not subject to cracking.

Because of the above mentioned properties of columbium, it has been suggested to use this metal in the form of jet turbine blades and buckets, rocket nozzles, and the like, where such members are subjected to high temperature conditions and to great thermal and physical shock. However, substantially pure columbium metal is, for all practical purposes, non-utilizable as the material for such members because at high temperatures and in the presence of flowing air or in the presence of oxygen-containing corrosive gases for an extended period of time, the strength characteristics of the pure metal are too low and the pure metal oxidizes too rapidly.

In accordance with the present invention, there is provided a new and improved columbium alloy which not only retains all of the above mentioned desired properties of the pure columbium metal, but which, when compared with the pure metal, has unexpected and markedly improved strength characteristics and resistance to oxidation at elevated temperatures.

The columbium alloy of this invention is comprised of columbium and tungsten or molybdenum, or mixtures of tungsten and molybdenum. When tungsten is combined with columbium in the alloy of this invention, the alloy may contain from about 0.99 percent (0.5 atomic percent) to about 67 percent (50 atomic percent) of tungsten, the balance being substantially all columbium. When molybdenum is combined with columbium in the alloy of this invention, the alloy may contain from about 0.51 percent (0.5 atomic percent) to about 20.5 percent (20 atomic percent) of molybdenum, the balance being substantially all columbium. When the alloy of this invention is comprised of columbium and a mixture of tungsten and molybdenum, then the combined tungsten and molybdenum content may be from about .52 percent (0.5 atomic percent) to about 66.3 percent (50 atomic percent) with this proviso, the molybdenum content cannot exceed 20.5 percent (20 atomic percent).

The alloy and the powder employed to form the alloy are preferably held to a high purity standard. The carbon content in the final alloy is preferably held to 0.4 percent or less, the oxygen content to 0.8 percent or less, and the

2

nitrogen content to 0.2 percent or less. Columbium powder, with an analysis of 0.25 percent carbon, 0.010 percent silicon, 0.030 percent titanium and 0.005 percent iron has been used successfully with alloying metal powders of 99 percent purity.

The term "atomic percent" of an element as used herein means the percentage of the total number of atoms in a mass of the alloy which are atoms of that particular element. The term "percent" of an element as used herein means the percentage of the total weight of a mass of the alloy which is the weight of that particular element.

Following are examples of the preparation and test results of columbium alloys of this invention:

## Example I

15 A columbium alloy composition of 99.01 percent (99.5 atomic percent) columbium and 0.99 percent (0.5 atomic percent) tungsten was prepared by arc melting an electrode of columbium to which 0.99 percent tungsten was added during melting. This may be accomplished by spot-welding the required amount of tungsten in strip form to the columbium electrode and then arc melting the assembly in helium. It also may be accomplished by arc melting a composite electrode consisting of a pressed and presintered powder blend of the required amounts of columbium and tungsten, in helium. This electrode may be prepared by pressing a blend of powders of the metals at a pressure of 50 t.s.i. to form a green compact which may then be presintered at a temperature of about 2000° C. for about two hours in a vacuum of about 1 or 2 microns. Other conventional presintering conditions may be used.

The arc melting procedures may be carried out in argon, a mixture of argon and helium, or in other inert gas.

35 The resulting arc melted alloy when tested for oxidation resistance in air at 2000° F. for sixteen hours is markedly superior in resistance to oxidation compared to unalloyed arc melted columbium metal.

40 In determining the oxidation rate, the dimensions of the test sample were determined prior to subjecting the sample to the oxidizing test conditions, the oxide film which formed on the surface of the test sample was removed, as by grit blasting or grinding, following which the thickness of the sample was measured. The change in dimension affords the means of measuring the amount of metal lost by oxidation during the test period. It is to be noted that the difference between the thickness of the original test sample and the thickness following exposure to an oxidizing atmosphere is referred to as "oxidation penetration" into the metal.

45 The columbium base alloy of this example is about one and one-half (1½) times greater in strength than unalloyed arc melted columbium metal, as determined by resistance to deformation at elevated temperatures of 2000° F. to 2200° F.

50 In determining the strength characteristics, test samples of the alloys were subjected to predetermined elevated temperature conditions in an oxidizing atmosphere and the sample loaded to a given stress condition. The degree of deformation as a function of time was noted, and this is referred to herein as "resistance to deformation."

## Example II

55 A columbium alloy consisting of 94.3 percent (97 atomic percent) columbium and 5.7 percent (3 atomic percent) tungsten was prepared by arc melting a presintered electrode made from the indicated amounts of the metals as described in Example I, in a mixture of helium and argon.

60 The resulting arc melted columbium alloy when tested for oxidation resistance in air by subjecting a test speci-

men to the atmosphere at 2000° F. for a period of sixteen hours underwent an oxidation penetration of 0.015 cm.

This result is to be compared with an oxidation penetration of 0.085 cm. for unalloyed arc melted columbium subjected to the same conditions for the same period of time.

The strength of this alloy is two (2) times as great as unalloyed arc melted columbium metal tested under the same conditions, based on resistance to deformation of test specimens at elevated temperatures of between 2000° F. and 2200° F.

### Example III

A columbium alloy composition consisting of approximately 90.6 percent (95 atomic percent) columbium and 9.4 percent (5 atomic percent) tungsten was prepared by powder metallurgy technique wherein 2000 grams of columbium powder and 207 grams of tungsten powder were intimately mixed and blended and the resulting powder mix pressed and sintered into an alloy bar. The blend was pressed at a pressure of 50 t.s.i. to form a green compact which was then sintered at a temperature of about 2000° F. for about two hours in a vacuum of about 1 or 2 microns.

A test specimen of this alloy bar when tested for oxidation resistance in air at 2000° F. for sixteen hours underwent an oxidation penetration of 0.013 cm. This compares with an oxidation penetration of 0.085 cm. for unalloyed arc melted columbium, subjected to the same conditions for the same period of time.

Another test specimen from this alloy when tested for strength characteristics based on resistance to deformation at elevated temperatures of between 2000° F. to 2200° F. showed that this alloy has two and one-half (2½) times the strength of unalloyed arc melted columbium metal tested under the same conditions.

### Example IV

A columbium alloy consisting of 82 percent (90 atomic percent) columbium and 18 percent (10 atomic percent) tungsten was prepared by arc melting a presintered electrode made from the indicated amounts of the metals as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of 0.010 cm. and when subjected for a period of sixty-six hours, underwent an oxidation penetration of 0.090 cm. On the other hand, unalloyed arc melted columbium when subjected to the same conditions for sixteen hours undergoes an oxidation penetration of 0.085 cm. and for sixty-six hours undergoes an oxidation penetration of 0.345 cm.

Another test specimen from this alloy, when tested for strength characteristics based on resistance to deformation at elevated temperatures of 2000° F. to 2200° F., showed that this alloy has three (3) times the strength of unalloyed arc melted columbium metal tested under the same conditions.

### Example V

A columbium alloy consisting of 67 percent (80 atomic percent) columbium and 33 percent (20 atomic percent) tungsten was prepared by arc melting a presintered electrode made from the indicated amounts of the metals as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of 0.005 cm. This result is to be compared with an oxidation penetration of 0.085 cm. for unalloyed arc melted columbium subjected to the same test conditions for the same period of time.

The strength of this alloy is at least three and one-half (3½) times as great as unalloyed arc melted columbium metal tested under the same conditions. The strength tests were based on resistance to deformation of test specimens at elevated temperatures of 2000° F. to 2200° F.

### Example VI

A columbium alloy consisting of 54.2 percent (70 atomic percent) columbium and 45.8 percent (30 atomic percent) tungsten was prepared by arc melting a presintered electrode of the indicated amounts of the metals made as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of 0.002 cm. and when subjected to the same conditions for sixty-six hours underwent an oxidation penetration of 0.039 cm. Unalloyed arc melted columbium when tested under the same conditions for sixteen hours undergoes an oxidation penetration of 0.085 cm. and for sixty-six hours undergoes an oxidation penetration of 0.354 cm.

The strength of this alloy is at least three and three-quarter (3¾) times as great as unalloyed arc melted columbium metal tested under the same conditions. These tests were based on resistance to deformation of test specimens at elevated temperatures of 2000° F. to 2200° F.

### Example VII

A columbium alloy consisting of 33 percent (50 atomic percent) columbium and 67 percent (50 atomic percent) tungsten was prepared by arc melting a presintered electrode of the indicated amounts of the metals made as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of 0.001 cm. This result is to be compared with an oxidation penetration of 0.085 cm. for unalloyed arc melted columbium subjected to the same test conditions for the same period of time.

The strength of this alloy is at least four (4) times as great as unalloyed arc melted columbium metal tested under the same conditions. These tests were based on resistance to deformation of test specimens at elevated temperatures of 2000° F. to 2200° F.

### Example VIII

A columbium alloy composition of 99.49 percent (99.5 atomic percent) columbium and 0.51 percent (0.5 atomic percent) molybdenum was prepared by arc melting a presintered electrode of the indicated amounts of the metals made as described in Example I, in a mixture of helium and argon.

The resulting arc melted alloy when tested for oxidation resistance in air at 2000° F. for sixteen hours was markedly superior in resistance to oxidation to unalloyed arc melted columbium metal.

This alloy is about one and one-half (1½) times greater in strength than unalloyed arc melted columbium as determined by resistance to deformation at an elevated temperature of 2000° F. to 2200° F.

### Example IX

A columbium alloy consisting of 96.9 percent (97 atomic percent) columbium and 3.1 percent (3 atomic percent) molybdenum was prepared by arc melting a presintered electrode of the indicated amounts of the metals made as described in Example I, in a mixture of helium and argon.

The resulting arc melted columbium alloy when tested for oxidation resistance in air by subjecting a test specimen to the atmosphere at 2000° F. for a period of sixteen

hours underwent an oxidation penetration of 0.019 cm. This result is to be compared with an oxidation penetration of 0.085 cm. for unalloyed arc melted columbium subjected to the same test conditions for the same period of time.

The strength of this alloy is at least two (2) times as great as unalloyed arc melted columbium metal tested under the same conditions. These tests were based on resistance to deformation at elevated temperatures of 2000° F. to 2200° F.

#### Example X

A columbium alloy consisting of 89.7 percent (90 atomic percent) columbium and 10.3 percent (10 atomic percent) molybdenum was prepared by arc melting a presintered electrode of the indicated amounts of the metals made as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of 0.012 cm. This result is to be compared with an oxidation penetration of 0.085 cm. for unalloyed arc melted columbium.

The strength of this alloy is at least two and one-half (2½) times as great as unalloyed arc melted columbium metal tested under the same conditions. These tests were based on resistance to deformation of test specimens at elevated temperatures of 2000° F. to 2200° F.

#### Example XI

A columbium alloy consisting of 79.5 percent (80 atomic percent) columbium and 20.5 percent (20 atomic percent) molybdenum was prepared by arc melting a presintered electrode of the indicated amounts of the metals made as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of 0.008 cm. This result is to be compared with an oxidation penetration of 0.085 cm. for unalloyed arc melted columbium.

The strength of this alloy is at least two and three-quarter (2¾) times as great as unalloyed arc melted columbium metal tested under the same conditions. These tests were based on resistance to deformation of test specimens at elevated temperatures of 2000° F. to 2200° F.

A preferred range of alloying constituents in the columbium base alloy of this invention is from about 18 percent (10 atomic percent) to about 45.8 percent (30 atomic percent) tungsten, the balance being substantially all columbium. When molybdenum is substituted for tungsten in the columbium base alloy of this invention the preferred range is from about 10.3 percent (10 atomic percent) to about 20.5 percent (20 atomic percent) molybdenum, the balance being substantially all columbium.

Alloys comprising from about 0.52 percent (0.51 atomic percent) to about 66.9 percent (49.9 atomic percent) of a mixture of tungsten and molybdenum, the balance being substantially all columbium have the desired properties of oxidation resistance and high strength at elevated temperatures as the alloys of the foregoing examples.

It is important to note that the molybdenum content of the columbium-tungsten-molybdenum alloy should be no greater than 20 atomic percent of the alloy.

It has been found that the oxidation resistance of the alloys of this invention (columbium-tungsten, columbium-molybdenum, or columbium-tungsten-molybdenum) as well as the strength characteristics, may be further improved by incorporating in the alloys from about 0.1 percent to 2 percent silicon or 0.1 percent to 2.0 percent aluminum, as well as mixtures of these metals, wherein the total weight of the combined aluminum and silicon

does not exceed 2.0 percent in the columbium base alloy. Following are examples of the preparation and test results of columbium base alloys of this invention incorporating silicon and aluminum.

#### Example XII

A columbium base alloy consisting of 65.55 percent (77 atomic percent) columbium, 33.7 percent (20 atomic percent) tungsten, and .75 percent (3 atomic percent) aluminum in the form of aluminum columbide ( $Al_3Cb$ ) was made by arc melting a presintered electrode made from the indicated amounts of these materials as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of .0035 cm. This result is to be compared with an oxidation penetration of 0.085 cm. for unalloyed arc melted columbium.

The strength of this alloy is at least three and one-half (3½) times as great as unalloyed arc melted columbium metal tested under the same conditions. These tests were based on resistance to deformation of test specimens at elevated temperatures of 2000° F. to 2200° F.

#### Example XIII

A columbium alloy consisting of 65.63 percent (77 atomic percent) columbium, 33.6 percent (20 atomic percent) tungsten, and .77 percent (3 atomic percent) silicon was prepared by arc melting a presintered electrode made from the indicated amounts of these metals as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of 0.0035 cm. This result is to be compared with an oxidation penetration of 0.085 cm. for unalloyed arc melted columbium.

The strength of this alloy is at least three and one-half (3½) times as great as unalloyed arc melted columbium metal tested under the same conditions. These tests were based on resistance to deformation of test specimens at elevated temperatures of 2000° F. to 2200° F.

To the columbium-tungsten, columbium-molybdenum, columbium-tungsten-molybdenum alloys of this invention may be added titanium in an amount of from 2 percent to 20 percent of the alloy. As a result of the addition of titanium to the alloy of this invention in the stated proportions the strength and oxidation resistance of the alloy is retained, but the density is lowered. This is of particular importance where the alloys of this invention are to be used as structural material in turbine blades for aircraft where maximum oxidation and strength requirements are desired, but concomitant therewith the lowest possible density is required.

Following are examples of the preparation and test results of columbium base alloys of this invention incorporating titanium.

#### Example XIV

A columbium alloy consisting of 75 percent (68 atomic percent) columbium, 10 percent (5 atomic percent) tungsten and 15 percent (27 atomic percent) titanium was made by arc melting a presintered electrode made from the indicated amounts of these metals as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of 0.057 cm. This result is to be compared with an oxidation penetration of 0.085 cm. for unalloyed arc melted columbium.

The strength of this alloy is at least two (2) times as great as unalloyed arc melted columbium metal tested under the same conditions. These tests were based on resistance to deformation of test specimens at elevated temperatures of 2000° F. to 2200° F.

*Example XV*

A columbium alloy consisting of 68 percent (67 atomic percent) columbium, 20 percent (10 atomic percent) tungsten, and 12 percent (23 atomic percent) titanium was prepared by arc melting a presintered electrode made from the indicated amounts of these metals as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of 0.023 cm. This result is to be compared with an oxidation penetration of 0.085 cm. for unalloyed arc melted columbium.

The strength of this alloy is at least two and one-half (2½) times as great as unalloyed arc melted columbium metal tested under the same conditions. These tests were based on resistance to deformation of test specimens at elevated temperatures of 2000° F. to 2200° F.

*Example XVI*

A columbium alloy consisting of 86.8 percent (86 atomic percent) columbium, 8 percent (4 atomic percent) tungsten and 5.2 percent (10 atomic percent) titanium was prepared by arc melting a presintered electrode made from the indicated amounts of the metals as described in Example I, in a mixture of helium and argon.

The resulting arc melted columbium alloy when tested for oxidation resistance in air by subjecting a test specimen to the atmosphere at 2000° F. for a period of sixteen hours underwent an oxidation penetration of 0.011 cm. This result is to be compared with an oxidation penetration of 0.085 cm. for unalloyed arc melted columbium.

The strength of this alloy is at least two (2) times as great as unalloyed arc melted columbium metal tested under the same conditions. These tests were based on resistance to deformation of test specimens at elevated temperatures of 2000° F. to 2200° F.

The strength characteristics of the alloys comprised of columbium, tungsten and titanium, columbium, molybdenum and titanium, and columbium, tungsten, molybdenum and titanium, may be further improved by incorporating in the alloys from 0.1 percent to 2.0 percent silicon or 0.1 percent to 2.0 percent aluminum, as well as mixtures of these metals, wherein the total weight of the combined aluminum and silicon does not exceed 2.0 percent in the columbium base alloy.

Following is an example of a columbium base alloy of this invention incorporating tungsten, molybdenum, titanium, and silicon and aluminum.

*Example XVII*

A columbium alloy consisting of 86.6 percent (80 atomic percent) columbium, 4.3 percent (2 atomic percent) tungsten, 2.2 percent (2 atomic percent) molybdenum, 5.6 percent (10 atomic percent) titanium, .7 percent (2 atomic percent) silicon and .6 percent (2 atomic percent) aluminum was prepared by arc melting a presintered electrode made from the indicated amounts of the metals as described in Example I, in an atmosphere of a mixture of helium and argon gases.

The resulting arc melted columbium alloy when tested for oxidation resistance in air by subjecting a test specimen to the atmosphere at 2000° F. for a period of sixteen hours underwent an oxidation penetration of 0.009 cm. This result is to be compared with an oxidation penetration of 0.085 cm. for unalloyed arc melted columbium.

The strength of this alloy is at least two and one-half

(2½) times as great as unalloyed arc melted columbium metal tested under the same conditions. These tests were based on resistance to deformation at elevated temperatures of 2000° F. to 2200° F.

The foregoing detailed description is given for clearness of understanding of the invention, and no unnecessary limitations should be understood therefrom, for some modification will be obvious to those skilled in the art.

We claim:

1. A columbium alloy which is composed essentially of: columbium and tungsten, there being from about 0.99 percent to about 67 percent tungsten and the balance being substantially all columbium.
2. A columbium alloy which is composed essentially of: columbium and tungsten, there being from about 18 percent to about 45.8 percent of tungsten, the balance being substantially all columbium.
3. A columbium alloy which is composed essentially of: columbium; a metal selected from the group consisting of tungsten, molybdenum, and mixtures thereof, the content of tungsten when selected being from about 0.99 percent to about 67 percent, the content of molybdenum when selected being from about 0.51 percent to about 20.5 percent, and the content of mixtures of tungsten and molybdenum when selected being from about 0.52 percent to about 66.3 percent, the maximum molybdenum being about 20.5 percent; and from about 2 percent to about 20 percent titanium; the balance being substantially all columbium.
4. A high temperature ternary alloy composed of, by weight: about 50 to 70% niobium, about 15 to 30% tungsten, and about 2 to 15% titanium.
5. A high temperature alloy consisting essentially of by weight about 10 to 30% tungsten, 2 to 15% titanium, up to 15% molybdenum, and the balance being essentially columbium.
6. A high temperature alloy consisting essentially of by weight about 0.2% to 2% aluminum, about 4% to 15% molybdenum, and the balance being essentially columbium.
7. A columbium base alloy consisting essentially of by weight about 9-11% molybdenum, about 3-7% titanium, about 10% tungsten, about 0.5-2% aluminum and the balance substantially all columbium.

45

*References Cited by the Examiner*

UNITED STATES PATENTS

- |           |        |               |          |
|-----------|--------|---------------|----------|
| 1,811,487 | 6/1931 | Belding       | 75-174   |
| 2,754,203 | 7/1956 | Vordahl       | 75-175.5 |
| 2,754,204 | 7/1956 | Jaffee et al. | 75-175.5 |
| 2,822,268 | 2/1958 | Hix           | 75-174   |
| 2,838,395 | 6/1958 | Rhodin        | 75-174   |
| 2,838,396 | 6/1958 | Rhodin        | 75-174   |

55

OTHER REFERENCES

H. Buckle: "Structure and Microhardness of Binary and Ternary Systems of the Metals Columbium, Tantalum, Molybdenum, and Tungsten," Metallforschung, vol. 1, 1946, pp. 53-56 relied on.

60 "Initial Investigation of Niobium and Niobium-Base Alloy," Saller et al., U.S. Atomic Energy Commission report, May 23, 1955.

Journal of Metals, May 1952, p. 516.

65 Titanium Symposium, Papers 12 and 13, Department of the Navy, Office of Naval Research, Washington, D.C., Dec. 16, 1948.

DAVID L. RECK, Primary Examiner.

70 CLAUDE A. LEROY, MARCUS U. LYONS, NATHAN MARMELSTEIN, RAY K. WINDHAM, HYLAND BIZOT, Examiners.

N. A. RAUTIOLA, W. B. NOLL, W. C. TOWNSEND, C. N. LOVELL, Assistant Examiners.

75